

## UNITED STATES PATENT OFFICE.

JOSEPH SLEPIAN, OF WILKINSBURG, PENNSYLVANIA, ASSIGNOR TO WESTINGHOUSE ELECTRIC & MANUFACTURING COMPANY, A CORPORATION OF PENNSYLVANIA.

## MEANS FOR PREVENTING OCCLUSION OF HYDROGEN IN METAL CATHODES.

No Drawing.

Application filed January 12, 1920. Serial No. 351,005.

*To all whom it may concern:*

Be it known that I, JOSEPH SLEPIAN, a citizen of the United States, and a resident of Wilkinsburg, in the county of Allegheny 5 and State of Pennsylvania, have invented a new and useful Improvement in Means for Preventing Occlusion of Hydrogen in Metal Cathodes, of which the following is a specification.

10 My invention relates to electrolytic reactions and methods of conducting them, and it has, for its primary object, the provision of a method by which the occlusion of gases, and, particularly, of hydrogen in metallic 15 electrodes, to any material extent is prevented.

Heretofore, for some purposes, considerable difficulty has been experienced in electro-plating steel and other ferrous metals 20 because of the deleterious effect upon such metals occasioned by occluded gases and, particularly, hydrogen which may have been absorbed by them during the electro-plating treatment. The primary object of my present invention, therefore, resides in the provision of a method of electro-plating ferrous bodies or articles in such manner as to 25 prevent, to as great an extent as possible, any occlusion of gases in the metals being treated.

I have observed that, when employing metallic electrodes in a suitable electrolyte, in the nature of a cold solution, even very small currents would produce gas at the electrodes, and the electrolyte, on this account, would offer an abnormal resistance to the 35 passage of current. As the solution warmed up, however, I noted that the gases disappeared and that, between the temperature of 40 between 30 and 35° C., the gassing ceased and the resistance became normal, even for relatively high current densities.

In my opinion, this may be accounted for by assuming that, when hydrogen is liberated, in gaseous form, from a solution, by 45 an electric current, it cannot be returned into solution by reversals of the current, because the gas thus liberated is a non-conductor. If, however, the hydrogen ions are occluded by the metallic electrodes employed, they then act like conducting varieties of 50 hydrogen and will return into the solution or electrolyte upon reversal of the current.

If the foregoing theory is correct, and all 55 tests conducted by me indicate that it is, it

will be clear that gas occlusion in metallic electrodes, and, particularly, in ferrous electrodes, such as steel, increases rapidly with the temperature of the electrolyte and especially when such temperature approaches 60 30° C.

My present invention, therefore, resides in conducting electrolytic reactions of this character under such conditions as to maintain the electrolyte employed in a cool condition, in order that the ferrous electrodes being treated may not absorb the hydrogen or the other gases which may be given off. For example, in practising my invention, I may dispose ferrous or steel electrodes in a 70 proper electro-plating bath or electrolyte and I may pass a suitable current between the electrodes through the bath while maintaining the bath in a cool state by any suitable means, as by the employment of cooling 75 coils immersed in the bath. Although I do not wish to be restricted to specific details, the primary feature of my invention resides in keeping the temperature of the bath below 30° C., and, preferably, in keeping the 80 bath relatively cool.

In practising my invention, I may provide a solution of approximately 1% sodium carbonate in water and utilize electrodes of ingot iron of suitable size. The electrolysis 85 may be carried out with a current density of  $\frac{1}{2}$  to 10 amperes per square inch at 25 cycles A. C. The temperature is preferably maintained below 30° C.

While it is not essential, I prefer to practise my invention under a reduced pressure, as this is also beneficial in keeping the gases from going into the metallic electrodes. In view of the relatively broad scope of my invention, including, as it does, the employment 95 of numerous characters of electrodes and electrolytic solutions, it will be appreciated that no limitations are to be imposed upon my invention other than those indicated in the appended claims.

100 I claim as my invention:—

1. The method of preventing occlusion of gases in ferrous electrodes of electrolytic apparatus that comprises maintaining the electrolyte employed in a cool state.
2. The method of preventing occlusion of gases in iron being treated during electro-plating that comprises keeping the electrolytic bath at a temperature below 30° C.
3. The method of preventing occlusion of 110

gases in iron being treated during electro-plating that comprises keeping the electrolytic bath at a temperature below 30° C., and carrying out the operation under sub-  
5 atmospheric pressure.

4. The method of preventing occlusion of gases in ferrous electrodes of electrolytic ap-

paratus that comprises maintaining the electrolyte employed in a cool state and electrolyzing with an alternating current.

In testimony whereof, I have hereunto subscribed my name this 31st day of December, 1919.

JOSEPH SLEPIAN.